

## 1

3,249,465

### METHOD OF IMPROVING THE HYDROPHILICITY OF POLYURETHANE CELLULAR PRODUCT AND THE RESULTING PRODUCT

Ming Chih Chen, Park Forest, Ill., assignor to Simoniz Company, a corporation of Delaware  
No Drawing. Filed Aug. 18, 1961, Ser. No. 132,318  
7 Claims. (Cl. 117—98)

This invention relates to the method of improving the hydrophilic properties of polyurethane sponge materials and to the resulting product.

This application is a continuation-in-part of my pending application Serial No. 752,437, filed August 1, 1958, now abandoned.

Organic foam sponges with interconnecting pores are useful as cleaning articles in washing and scrubbing surfaces. The ideal sponge should not only be capable of absorbing large amounts of water and to hold the water for use during the cleaning operation but should also be easily wet with water. The different types of sponges available for cleaning uses have been somewhat limited. With the product and process of this invention it is now possible to produce excellent hydrophilic polyurethane sponges (which are normally hydrophobic) that are useful as cleaning articles.

In general, the method of this invention comprises soaking the polyurethane sponge material in an aqueous dispersion of a hydrophilic agent that is essentially water insoluble but water dispersible. The concentration in the aqueous liquid of the agent should be less than that which would damage the sponge material. This amount will vary with the different agents and with the different polyurethanes but is easily determined as an excess concentration has a solvent and weakening action on the urethane material.

The liquid in which the hydrophilic agent is dispersed may be water or may be an aqueous solution or dispersion of a swelling agent for the polyurethane with these swelling agents being well known in the art and including aliphatic alcohols, ketones, ethers, halogenated hydrocarbons and the like. In general, the treating bath should not contain, of course, such an amount of the swelling agent that the sponge is excessively weakened.

The temperature of the treating bath must be above room temperature where no swelling agent is present but may be as low as room temperature where a swelling agent is present. A preferred temperature of the bath is about 20–85° C. with the temperature being preferably in the bottom portion of the range (for example, about 20–45° C.) when a swelling agent or solvent for the urethane is present and in the remainder of the range when the bath is substantially water. The urethane is maintained in contact with the bath until the material has been completely wetted and retains at least about 1% of the hydrophilic agent by weight on a dry basis.

## 2

More specifically, the method of this invention comprises soaking the polyurethane sponge material with a dispersion in a liquid carrier containing about 0.1% or higher, but preferably from about 1–3%, by weight of an essentially water insoluble but water dispersible hydrophilic agent at a temperature of about 20–85° C., and preferably about 55–65° C., for a time sufficient to thoroughly wet the polyurethane sponge and to retain at least about 1%, but preferably about 5–20%, by weight of the hydrophilic agent based on the weight of the sponge on a dry basis. Where substantially no swelling agent is present the temperature should preferably be about 45–85° C. In ordinary commercial practice the time can vary from about 1 second to about 24 hours. At the end of this time the excess liquid is removed from the sponge material as by squeezing.

The resulting treated polyurethane sponge is found to be relatively hydrophilic and capable of being more easily wet with water than was the untreated sponge. The method of this invention can be used either on polyester urethanes or polyether urethanes and both types will be converted from a hydrophobic condition to a relatively hydrophilic condition. The preparations of typical polyurethanes are disclosed in numerous U.S. and foreign patents and publications. Many are disclosed in my co-pending U.S. patent application Serial No. 74,463, filed December 8, 1960, now abandoned, and particularly at pages 10 to 21 thereof. The hydrophilic agents that are preferred in this invention are those that are essentially water insoluble but self-dispersible. Highly water soluble agents such as those of infinite solubility are not used because they lose their effectiveness on long rinsing of the treated sponge. Thus, the "essentially" water insoluble agents may be slightly water soluble but water dispersible and still be usable. Oil soluble and substantially completely water insoluble hydrophilic agents are dispersed in the water by means of a dispersing agent.

It has been observed during the soaking of the sponge in a bath containing the hydrophilic agent that the sponge actually absorbs the hydrophilic agent from the bath, thus reducing the concentration of the agent in the bath as contact time increases. The bath can be made either with water or with water having an organic solvent for the agent dispersed therein. Typical solvents are low molecular weight ketones, low molecular weight aliphatic alcohols, low molecular weight aliphatic ethers and the like. Thus, a suitable bath has been found to be made up of 40–95% water and 5–60% methanol by weight. This illustrates those instances where the dispersing agent (e.g. methanol) for the essentially water insoluble hydrophilic agent also acts as a swelling agent for the sponge material.

Among the hydrophilic agents that have been found especially suitable for the method of this invention are the following:

| No.    | Agent                | Chemical Composition                                                                                                                        |
|--------|----------------------|---------------------------------------------------------------------------------------------------------------------------------------------|
| 1..... | Ninol H.A.10.....    | Coconut diethanol amide.                                                                                                                    |
| 2..... | Makon 6.....         | Reaction product of one mole nonyl phenol and 6 moles of ethylene oxide.                                                                    |
| 3..... | Dispersant NI-O..... | Reaction product of one mole alkyl phenols containing $C_{12}-C_{18}$ (average $C_{15}$ ) in the alkyl groups and 4–5 moles ethylene oxide. |
| 4..... | Renex 36.....        | Reaction product of one mole tridecyl-alcohol and 6 moles of ethylene oxide.                                                                |
| 5..... | Triton X-155.....    | Reaction product of one mole octyl phenol and 5–7 moles of ethylene oxide.                                                                  |

| No. | Agent           | Chemical Composition                                                                                                                                                |
|-----|-----------------|---------------------------------------------------------------------------------------------------------------------------------------------------------------------|
| 6   | Alkaterge A     |                                                                                                                                                                     |
| 7   | Alkaterge E     |                                                                                                                                                                     |
| 8   | Alkaterge C     |                                                                                                                                                                     |
| 9   | Alkaterge T     |                                                                                                                                                                     |
| 10  | Dispersant NL-E | Reaction product of one mole alkyl phenols containing C <sub>12</sub> -C <sub>16</sub> (average C <sub>15</sub> ) in the alkyl groups and 3-4 moles ethylene oxide. |
| 11  | Triton X-114    | Reaction product of one mole t-octyl phenol and 7 to 8 moles of ethylene oxide.<br>                                                                                 |
| 12  | Triton X-45     | Reaction product of one mole t-octyl phenol and 5 moles of ethylene oxide.                                                                                          |
| 13  | E <sub>1</sub>  | Reaction product of one mole tallow alcohol and 2 moles ethylene oxide, average alkyl carbon chain length of C <sub>16</sub> to C <sub>18</sub> .                   |
| 14  | E <sub>2</sub>  | Reaction product of one mole tallow alcohol and 4 moles ethylene oxide, average alkyl carbon chain length of C <sub>16</sub> to C <sub>18</sub> .                   |
| 15  | Amidox C2       | Ethoxylated alkylol-amide of essentially the formula:<br>$C_{12}H_{25}CON(C_2H_4OC_2H_4OH)_2$                                                                       |
| 16  | Triton N57      | Nonyl phenoxy polyethoxy ethanol of essentially the formula:<br>                                                                                                    |

The usable hydrophilic agents of which the above list is exemplary are either oil soluble (soluble in organic solvents) or essentially water insoluble but water dispersible either with a dispersing agent such as methanol or even without a dispersing agent in some instances. This insures their retention in the foam or sponge (terms used herein interchangeably) without premature loss of hydrophilic characteristics. Water dispersions of those self-dispersing hydrophilic agents are easily made by merely adding them to the water. However, if the material is oil soluble such as agents 6-8 of the above list, it will not disperse in water without the addition of a dispersing agent. In order to disperse this type of material in water an additional dispersing agent such as Tergitol NPX (a reaction product of one mole nonyl phenol and 10 moles of ethylene oxide) should be used or if desired a mixture of alcohol and water can be used as a dispersant.

As pointed out above, the sponges that are treated by the method of this invention may be any of the poly-ester or polyether urethanes. Whether in the form of a sponge or a sheet the urethane are rendered hydrophilic by the method of this invention. Typical methods of making polyurethanes are disclosed in my above-mentioned copending application Serial No. 74,463, and these are exemplary only.

A polyol polyurethane sponge prepared by Example 1 of my U.S. application Serial No. 74,463 was prepared as follows:

A prepolymer resin was prepared by the following

procedure: 444.8 lbs. of Pluronic L-61, hydroxyl number 50.5, was premixed with 63.5 lbs. of PPG-400, hydroxyl number 288.8, representing a hydroxyl equivalent ratio of 0.4448 to 0.3635. This polyol mixture should have a hydroxyl number of 80-81 and the acid number was adjusted to .03 and water content to 0.39%. To this mixture 235 lbs. of toluene diisocyanate, .002 to .003% total acidity, were added while mixing. The NCO/OH ratio was about 3.44. After 30 minutes the heat of reaction caused the temperature to rise to about 130° F. With additional heating requiring 2 hours, the mixture reached a temperature of 212° F. The reaction was allowed to proceed at 212° F. until the viscosity was about 3900-4200 centistokes. The resulting prepolymer was cooled to 100-125° F. It contained about 9.35% free NCO. The total process took about 8½ to 9½ hours.

For each 100 parts by weight of the above prepolymer, previously adjusted to 9.8% free NCO, the following were added: 0.2 part of silicone fluid DC-200 (polydimethylsiloxane) at 25° C. 50 centistokes viscosity, 17 parts Titanox RCHT-X and .167 part Benzedine Yellow No. 12220 dye.

A catalyst solution was made as follows: 15 parts water 1.5 parts triethyl amine and 5 parts diethylethanol amine.

The sponge material was prepared by foaming as follows:

Precision metering pumps were used to pump out the prepolymer resin/catalyst solution in the ratio of 32-25:1

to a mixing head having a capacity of 100 ml. Six triple blade turbine mixers were employed using a mixing speed of 3400 r.p.m. To facilitate the resin pumping, the resin was heated to 120° F. The rate of pumping was about 5 pounds per minute. The mixed material was delivered to a box-shaped mold through a  $\frac{3}{8}$ " opening where foaming took place immediately. After approximately 10 minutes, the foam's rise discontinued. After 30 minutes, it was removed from the mold and crushed by running between closely spaced squeeze rollers to break any closed cell walls, then postcured in a hot air oven at 185-190° F. for 16 hours. All said parts are by weight.

The Pluronic L-61 has the formula



It has a molecular weight of the polyoxypropylene base of about 1501-1800 and an oxyethylene content of about 10%. The PPG-400 is polypropylene glycol with a molecular weight of about 400. The Titanox RCHT-X consists of calcium sulfate particles coated with titanium dioxide.

A section 1" x  $\frac{3}{4}$ " x  $\frac{5}{8}$ " was cut from this sponge. Then a water dispersion was made up with 1.5% of hydrophilic agent No. 3 in the above list, all percentages being by weight. The section of sponge was saturated by this bath maintained at a temperature between 55-60° C. for about 10 minutes. Then the sponge was removed from the bath and wrung out. At the end of this time the sponge contained about 14.5% hydrophilic agent on the dry basis. Before this treatment the sponge had been found to float on water without wetting. As a result of this treatment the sponge became wet with water at a rate of less than 2 seconds per centimeter of thickness even after being rinsed with 2000 gallons of room temperature water at the rate of 500 gallons per hour.

Similar examples were performed using the polyurethanes prepared according to my above-mentioned application No. 74,463 and various of the hydrophilic agents in the above list. In every instance the polyurethane sponge material which before treatment had been hydrophobic was hydrophilic after the treatment. These examples were all performed within the conditions defined earlier in this application.

In other examples polyurethane foams were prepared according to Examples 2, 3, 4 and 5 of the above-mentioned application 74,463. Also, 1.5% aqueous dispersions of hydrophilic agents 2, 4, 5 and 11 of the above list were prepared. Each of the polyurethanes was soaked in one of these dispersions at temperatures of about 40-60° C. for 10 minutes time. At the end of this time the excess dispersion was removed and the polyurethane was found to be highly hydrophilic.

Similar tests were run using hydrophilic agents 9, 13 and 14 of the above list with the above-designated polyurethanes. In each of these instances the hydrophilic agents were dissolved in methanol and diluted with water to give a dispersion concentration of 1.5% of the agent in a 5% methanol-95% water mixture. The sections of urethane sponge were soaked in these dispersions for about 10 minutes at 40-60° C. at the end of which time the excess dispersion was removed. The sponges likewise were found to be hydrophilic. In each of these tests sections of the above-described dimensions were used.

In all of these tests the polyurethane foam material remains hydrophilic even after being continuously rinsed with room temperature water for 24 hours.

The essentially water insoluble but water dispersible hydrophilic agents of this invention appear to function by a physical action and not a chemical action. Thus, they appear to operate regardless of their chemical structure so long as they are dispersible in water but not water soluble so that the effect will not be lost too rapidly on contact with water. Furthermore, the action of the usable hydrophilic agents does not appear to depend upon the ionic character of the agent. The important determina-

tion of whether a hydrophilic agent will work or not is that it be water insoluble in that the agent is not completely dissolved even in the minimum amount recited above which is at least about 0.1% by weight in the aqueous dispersion.

The swelling agents mentioned herein have a solvent action on the sponges and thus the terms swelling agents and solvents are used interchangeably herein. Among the dispersing agent for the non self-dispersible surface active agents are the solvents mentioned above. Thus, these dispersing agents may be water soluble, low molecular weight ketones, water soluble, low molecular weight alcohols, water soluble low molecular weight ethers and the like which also act as the swelling agents or solvents. The dispersing agents also include, however, water soluble surface active agents of which the above-described Tergitol NPX is an example. The dispersing of essentially water insoluble but water dispersible hydrophylic agents is well understood in the hydrophilic agent art, as this is frequently done in order that they can be used in an aqueous medium.

Having described my invention as related to the embodiments set out herein, it is my intention that the invention be not limited by any of the details of description, unless otherwise specified, but rather be construed broadly within its spirit and scope as set out in the accompanying claims.

I claim:

1. The method of improving the hydrophilicity of a 30 polyurethane foam material, comprising: preparing a dispersion of an essentially water insoluble but water dispersible hydrophilic agent in a bath of the class consisting of water and aqueous solutions of a dispersing agent for said hydrophilic agent, said bath containing at least about 1% by weight of said bath of said hydrophilic agent; saturating said material with said bath maintained at a temperature within the range of about 20-85° C. for a time sufficient for said foam material to absorb at least about 1% of said hydrophilic agent by weight 40 of the anhydrous foam material, said temperatures being the bottom of said range when said bath is said solution and in the remainder of the range when said bath is substantially water; and removing said material.

2. The method of improving the hydrophilicity of a 45 polyurethane foam material, comprising: preparing a dispersion of an essentially water insoluble but water dispersible hydrophilic agent in a bath of the class consisting of water and aqueous solutions of a dispersing agent for said hydrophilic agent, said bath containing at least about 1% by weight of said bath of said hydrophilic agent; saturating said material with said bath maintained at a temperature within the range of about 20-85° C. for a time sufficient to absorb about 5-20% of said hydrophilic agent by weight of the anhydrous foam material, said temperature being in the bottom of said range when said bath is said solution and in the remainder of the range when said bath is substantially water; and removing said material.

3. The method of improving the hydrophilicity of a 60 polyurethane foam material, comprising: preparing a dispersion of an essentially water insoluble but water dispersible hydrophilic agent in a bath of the class consisting of water and aqueous solutions of a dispersing agent for said hydrophilic agent, said bath containing at least about 1-2% by weight of said bath of said hydrophilic agent; saturating said material with said bath maintained at a temperature within the range of about 20-85° C. for a time sufficient to absorb about 5-20% of said hydrophilic agent by weight of the anhydrous foam material, said temperature being in the bottom of said range when said bath is said solution and in the remainder of the range when said bath is substantially water; and removing said material.

4. The method of improving the hydrophilicity of a 75 polyurethane foam material, comprising: preparing a

dispersion in an aqueous bath of at least about .1% by weight of said bath of the hydrophilic agent reaction product of one mole of an alkyl phenol containing 12-16 carbon atoms in the alkyl groups and 4-5 moles ethylene oxide; saturating said material with said bath maintained at a temperature within the range of about 20-85° C. for a time sufficient to absorb at least about 1% of said hydrophilic agent by weight of the anhydrous foam material; and removing said material.

5. A hydrophilic product comprising: a polyurethane foam material having internal pores; and at least 1% on an anhydrous weight basis of an essentially water insoluble but water dispersible hydrophilic agent absorbed therein.

6. The product of claim 5 wherein said amount is about 15 5-20%.

7. The product of claim 5 wherein said surface active agent is the reaction product of one mole of an alkyl phenol containing 12-16 carbon atoms in the alkyl groups and 4-5 moles ethylene oxide.

5

References Cited by the Examiner

UNITED STATES PATENTS

|           |        |               |       |           |
|-----------|--------|---------------|-------|-----------|
| 2,711,969 | 6/1955 | Abig          | ----- | 117-102   |
| 2,753,277 | 7/1956 | Smithers      | ----- | 117-138.8 |
| 2,900,278 | 8/1959 | Powers et al. | ----- | 117-98    |
| 2,920,983 | 1/1960 | Bugosh        | ----- | 117-98    |
| 3,102,825 | 9/1963 | Rogers et al. | ----- | 117-98    |

WILLIAM D. MARTIN, *Primary Examiner.*

RICHARD D. NEVIUS, *Examiner.*